

Dec. 18, 1934.

E. D. WILSON

1,985,006

PHOTOTUBE

Filed April 22, 1933

FIG. 1.



FIG. 2.



FIG. 3.



WITNESSES:

E. A. McElroy.  
R. W. Bailey.

INVENTOR

Earl D. Wilson.  
BY F. W. Leyde.  
ATTORNEY

## UNITED STATES PATENT OFFICE

1,985,006

## PHOTOTUBE

Earl D. Wilson, Wilkinsburg, Pa., assignor to  
 Westinghouse Electric & Manufacturing Company, East Pittsburgh, Pa., a corporation of Pennsylvania

Application April 22, 1933, Serial No. 667,494

4 Claims. (Cl. 250—27.5)

My invention relates to photo-tubes, and it has particular relation to photo-tubes super-sensitive to the central and blue color region of the visible spectrum.

5 An object of my invention is to provide a photo-tube which has a color sensitivity similar to that of the average human eye.

Photo-tubes heretofore have been designed to produce the maximum response to light without 10 consideration of the quality of this response in regard to the various colors. The result has been that photo-tubes of the prior art have been super-sensitive to the red region of the visible spectrum and have not been sensitive to the 15 other sections of the visible spectrum.

In my copending case on photo-sensitive apparatus, Serial No. 524,878, filed March 24, 1931, I have described apparatus for color matching. It required a photo-tube for this apparatus that 20 would be sensitive to colors in the same degree as the average human eye, in order that the colors might be matched as they appeared to the average human eye.

This invention has a particular application in 25 the apparatus described in the copending case, but it is not limited to such an application. It is apparent that such a photo-tube will have various applications in view of the fact that the tube responds in the same degree to colors as does the average human eye.

The novel features that I consider characteristic of my invention are set forth with particularity in the appended claims. The invention itself, however, both as to its organization and 35 its method of operation, together with additional objects and advantages thereof, will best be understood from the following description of a specific embodiment when read in connection with the accompanying drawing, in which:

40 Figure 1 is a front elevation partly in section of the preferred structure of a photo-tube constructed in accordance with my invention;

Fig. 2 is a view in side elevation partly in section of the photo-tube of Fig. 1; and;

45 Fig. 3 is a graph showing the color sensitivity of my photo-tube in comparison with that of the average human eye, and of the standard red sensitive photo-tubes of the prior art.

The preferred structure of the photo-tube as 50 illustrated in Figs. 1 and 2 consists of a suitable envelope of transparent glass 10 mounted upon the usual base 11 with the usual conductors 12, 13 and 14 extending through the press of the tube to the interior thereof. The press has preferably flat sides 15 and centrally supports the

connection to the anode which consists of one or more wires or rods 16, 17, preferably extending through the central portion of the tube. At its upper end the anode structure preferably supports a pellet or capsule 18. The cathode 19 may likewise be supported from the same press, and while this cathode may have various forms, it is preferable to utilize the semi-cylindrical form disclosed in the drawing, partially surrounding the major portion of the anode.

5 The pellet or capsule 18 generally has about 50 milligrams of material composed of one part caesium-dichromate to two parts of pure silicon. It should be capable of releasing 3 milligrams of caesium per square inch of cathode surface. The cathode may be of silver, or may have a pure silver surface. It is preferably constructed of solid silver 3 mils thick and has an area of 10 2 square inches. Approximately a square inch of lead oxide or stannous oxide in a binder such 15 as amyl acetate is painted upon the flat sides 20 of the press.

The tube is baked at a temperature of about 25 400° C. until the gases and vapors are driven out of the glass and a good vacuum is obtained therein. The tube is then cooled to room temperature and about four millimeters of pure oxygen is admitted. About 100 volts direct current is then applied across the electrodes and produces a glow-discharge that oxidizes the silver surface of the cathode until the oxide which 30 is first formed is broken down by the heat of the discharge. Complete deoxidation takes place in about 5 seconds. The oxygen is then pumped out and a fresh supply of oxygen is admitted to the same pressure and the cathode is 35 oxidized carefully until its color passes through a bright green into a reddish tinge. The tube is again exhausted. An induction coil is placed around the tube and the pellet is flashed by induction currents to produce caesium vapor. The tube is then baked at a temperature between 225° and 275° C. until the reaction is 40 completed between the silver oxide surface of the cathode and the caesium. This reaction is visibly indicated by the cathode turning to a uniform dull black color. The lead oxide or stannous oxide painted on the press is for the purpose of absorbing the excess caesium vapor. If the cathode has a bronze or coppery appearance, it indicates that there had been too much 45 caesium released in the tube.

The baking is continued until the caesium-oxide is almost completely broken down into higher oxides. This is visually indicated by the 50 55

cathode becoming quite light to an ivory or cream appearance. If the cathode surface breaks up into orange colored spots, this phenomena indicates the presence of too much initial caesium for the type of tube.

The tube is cooled and preferably argon is admitted at about 200 microns pressure. A glow-discharge, preferably at a current density not exceeding 30 milli-amperes is passed through the tube again from the anode to the cathode until by test the sensitivity rises to a maximum value. When this maximum value is reached, the discharge is then reversed so that it passes from the cathode to anode until the sensitivity rises to a new maximum. After this new maximum is reached the discharge is reversed again for a short period so that it passes from anode to cathode until the sensitivity reaches a stationary value. The tube is then sealed off, unless a vacuum photo-tube is desired, in which case the argon is pumped out and the tube sealed after a sufficient vacuum is obtained.

In Fig. 3 are disclosed curves showing the relative sensitivity in regard to wavelength of the eye A, a photo tube constructed according to my invention described herein B, and a photo-tube sensitive to the red region C. The vertical scale of the eye is not drawn to the same scale as that of the tubes for the sake of clearness. It will be noted that my tube has a maximum sensitivity in the blue and central region of the spectrum in place of in the red region.

Although I have shown and described a certain specific embodiment of my invention, I am aware that many modifications thereof are possible. My invention, therefore, is not to be restricted except insofar as is necessitated by the prior art and by the spirit of the appended claims.

I claim as my invention:

1. The method of forming an electrode for a photo-electric tube which comprises oxidizing an electrode having a silver surface, heating said electrode surface in caesium vapor until it loses its black color, cooling said electrode to about room temperature, and subjecting it to glow discharge. 5

2. The method of forming an electrode for a photo-electric tube which comprises oxidizing an 10 electrode having a silver surface, heating said electrode surface in caesium vapor until it loses its black color, cooling said electrode to about room temperature, and subjecting it to glow discharge in an argon atmosphere until its light 15 sensitivity rises to a maximum, then reversing the polarity of said discharge until the light sensitivity rises to a second maximum, and then again reversing the polarity of said discharge until said sensitivity becomes constant. 20

3. The method of making a silver-surfaced cathode of a photo-tube photo-sensitive which comprises oxidizing the surface of said cathode, releasing about said cathode substantially 3 milligrams of caesium per square inch of said cathode surface, and then baking said cathode until the reaction is complete between the silver oxide surface of the cathode and the caesium. 25

4. The method of making a silver-surfaced cathode of a photo-tube photo-sensitive which comprises oxidizing the surface of said cathode, releasing about said cathode substantially 3 milligrams of caesium per square inch of said cathode surface, baking said cathode until the reaction is complete between the silver oxide surface of the cathode and the caesium, and then passing a glow discharge to the cathode. 30 35

EARL D. WILSON. 40